

# UNITED STATES PATENT OFFICE.

ALBERT H. SCHLAEDEL, OF INDIANAPOLIS, INDIANA, ASSIGNOR TO GRAPHO-METAL PRODUCTS COMPANY, OF INDIANAPOLIS, INDIANA, A CORPORATION OF INDIANA.

## PLASTIC PACKING AND PROCESS OF MAKING SAME.

1,324,763.

Specification of Letters Patent.

Patented Dec. 9, 1919.

No Drawing.

Application filed December 7, 1915. Serial No. 65,456.

*To all whom it may concern:*

Be it known that I, ALBERT H. SCHLAEDEL, a citizen of the United States, residing at Indianapolis, in the county of Marion and 5 State of Indiana, have invented new and useful Improvements in Plastic Packings and Processes of Making Same, of which the following is a full, clear, concise, and exact description, of this specification.

10 My invention relates to improvements in the manufacture of packing, especially such as is used in piston packing and bearings and has for its object the utilization of a process by means of which a packing is obtained that has great lubricating value and 15 also one that will stand up when subjected to great wear.

A further object is the utilization of a process by means of which a cheap and efficient packing may be obtained.

These and such other objects as may hereinafter appear are attained by my process, which is fully described and claimed in the accompanying specification.

25 In carrying out my invention I first take an alloy in the nature of Babbitt or bearing metal, composed for instance of lead, iron, copper, etc., the principal metals being substantially in the following proportions:

30 Lead 85%, iron 5%, copper 5%, bismuth 5%. I am not limiting myself to any particular Babbitt metal or composition, but can utilize such as may be purchased in the open market in bars or pigs.

35 In connection with the Babbitt metal, I also use graphite, both powdered and flaked, which may be of the ordinary brand either natural or artificial, and also a waxy composition of pure beeswax or beeswax and 40 paraffin, all of which products may be purchased in the open market.

In the production of my material, I first melt the alloy to the proper temperature, between 900 and 1200 degrees Fahrenheit, 45 the alloy beginning to break down at the lower temperature and being at about its working point at the higher temperature.

A tank or vat is provided having a depth of water between 9 and 12 inches, at a temperature between 75 to 85 degrees. The metal or alloy is dropped from a height of 6 to 7 feet above the surface directly from the crucible, preferably using a flat spout so that the metal falls in a thin flat sheet,

the crucible during the pouring being kept 55 in constant motion so that the metal strikes the water in a separated form. The crucible also is preferably carried about over the surface of the tank as the metal falls so that the metal in the tank is laid in the shape 60 of a spiral in the bottom when this part of the operation is completed. This method prevents the piling up of the metal near the top or above the surface of the water and facilitates the manufacture of the most 65 efficient product. When the metal strikes the water a slight explosion takes place and the resulting product is the metal itself in a loculate or porous condition.

After the contents of the crucible has 70 been poured, the water is drawn off from the tank and the metal allowed to drain and then put in an oven to dry. At this time the bearing metal is in large and small masses in an extremely divided or loculate 75 condition, but in such a condition as to be practically held together in considerably large pieces.

The next step in the operation consists 80 in the grading of the material to size, depending upon the use to which it is to be put and the size of the packing rings to be filled.

Take, for instance, what is called the manufacture of a No. 4 product. The material in this case is passed through a No. 4 riddle which comprises a screen or sieve with one-fourth inch mesh, and the material is rubbed about and forced through the screen. The fine material that breaks 90 up is removed therefrom for other grades and the material graded to fit the condition for which it is to be used.

Pure beeswax or beeswax and paraffin is next melted in a suitable vessel and powdered graphite mixed in, in the proportion of eight ounces of beeswax or beeswax and paraffin and two ounces of powdered graphite, the material then having a dirty appearance and forming a black waxy mass. 95

Ten lbs. of loculate metal is then added and the material kept stirring all the time until it is properly mixed and a temperature of from 350 to 450 degrees Fahrenheit is reached. At about this temperature 105 or between 400 and 450 degrees Fahrenheit four ounces of flake graphite is added and the material put in a tumbler and tumbled

while the temperature is decreasing, and at the proper moment, while the wax is still shrinking and before it has reached its point of ultimate shrinkage, four additional 5 ounces of flake graphite is added, which is caught in and held by the wax as it is shrinking.

Prior to the addition of the last four 10 ounces the mixed wax and graphite both powdered and flaked has gone into the pores of the metal practically filling them, except so far as the final shrinking of the wax is concerned and consequently the last four 15 ounces of flake graphite is mainly caught in or embedded in the wax at the entrance to the pores or close to the surface of the metal and wax.

By the practice of this process, a product 20 is obtained that is of great commercial value. It is sufficiently hard to stand ordinary usage when confined between rings, and the wax and the graphite is so commingled with the excess of flaked graphite 25 on the outside as to give the very best results as a packing or lubricant.

Of course it is understood that I am not 30 limiting myself to the exact proportions given either or any of the materials nor to the specific temperatures, the main idea being that the proper combination of flaked and powdered graphite with the wax, with the addition or surplusage of flake and graphite at the end produces the desired result.

Having thus described my invention, what 35 I claim as new and desire to secure by Letters Patent is:

1. The process of making metallic packing 40 consisting in reducing a bearing metal to a loculate condition, substantially filling said metal with a waxy filler containing graphite and subsequently adding more graphite while the said filler is shrinking.

2. The process of making metallic packing 45 consisting in reducing a bearing metal to a loculate condition, substantially filling said metal with a waxy filler containing graphite at a high temperature, permitting the temperature to lower and adding thereto 50 more graphite while the temperature is lowering.

3. The process of making metallic packing 55 consisting in reducing a bearing metal to a loculate condition, substantially filling said metal with a waxy filler containing beeswax and graphite at a high temperature, permitting the temperature to lower and

adding thereto more graphite while the temperature is lowering.

4. The process of making metallic packing 60 consisting in reducing a bearing metal to a loculate condition, substantially filling said metal with a waxy filler containing beeswax and powdered graphite at a high temperature, permitting the temperature to lower and adding thereto more graphite 65 while the temperature is lowering.

5. The process of making metallic packing 70 consisting in reducing a bearing metal to a loculate condition, substantially filling said metal with a waxy filler containing graphite at a high temperature, permitting the temperature to lower and adding thereto 75 flake graphite while the temperature is lowering.

6. The process of making metallic packing 80 consisting in reducing a bearing metal to a loculate condition, substantially filling said metal with a waxy filler containing beeswax and powdered graphite at a high 85 temperature, permitting the temperature to lower and adding thereto flake graphite while the temperature is lowering.

7. The process of making metallic packing 90 consisting in reducing a bearing metal to a loculate condition, substantially filling said metal with a waxy filler containing beeswax and powdered graphite and flake graphite at a high temperature, permitting the temperature to lower and adding thereto 95 flake graphite while the temperature is lowering.

8. The process of making metallic packing 100 consisting in reducing a bearing metal to a loculate condition, substantially filling said metal, mixing with said metal a waxy filler containing beeswax and powdered graphite, adding to said mixture additional flake graphite while at a high temperature, the lowering of said temperature while said material is being mixed and the addition of more flake graphite just before the waxy filler has reached its ultimate point of shrinkage.

9. A new article of manufacture, a packing 105 comprising loculate bearing metal having its pores filled with a lubricant containing graphite and having a surplusage of graphite embedded in the outer face of said lubricant.

In witness whereof I have hereunto subscribed my name.

ALBERT H. SCHLAEDEL.